

May 20, 1924.

1,494,410

W. S. BIDLE

METHOD OF MAKING TROLLEY WHEELS

Filed May 10 1922

2 Sheets-Sheet 1



May 20, 1924.

1,494,410

W. S. BIDLE

METHOD OF MAKING TROLLEY WHEELS

Filed May 10, 1922

2 Sheets-Sheet 2



Inventor  
W.S. BIDLE  
Timu  
Wren  
Huron  
Attorneys

Patented May 20, 1924.

1,494,410

# UNITED STATES PATENT OFFICE.

WILLIAM S. BIDLE, OF CLEVELAND, OHIO, ASSIGNOR TO THE COPPER PRODUCTS FORGING COMPANY, OF CLEVELAND, OHIO, A CORPORATION OF OHIO.

## METHOD OF MAKING TROLLEY WHEELS.

Application filed May 10, 1922. Serial No. 559,703.

To all whom it may concern:

Be it known that I, WILLIAM S. BIDLE, a citizen of the United States, residing at Cleveland, in the county of Cuyahoga and State of Ohio, have invented certain new and useful Improvements in a Method of Making Trolley Wheels, of which the following is a specification.

The present invention has for its object 10 the making of a hardened copper trolley wheel in a simple and efficient way, the steps taken being an improvement on the method shown and described in my application filed on the 27th day of February, 15 1922, Serial No. 539,458.

According to that method, I produce a trolley wheel of pure or unalloyed copper by cold working operations involving the parting of a copper blank by the use of a 20 sharp-edged roller.

In the present instance, I avoid the use of a sharp parting roller and cutting tool in the initial operations, and modify the subsequent groove shaping steps so as to 25 cause the metal in the worked surfaces to flow together at the base of the groove in such a manner that any fissure or fault may be definitely localized and easily removed.

The formations of the product at different 30 stages is exemplified in the drawings annexed hereto, in which Fig. 1 is a side view of a copper blank and a parting roller as related at the beginning of parting operations, and Fig. 2 is an edge elevation of the 35 parting roller and a sectional view of the blank and its holding dies in the same working relation. Figs. 3 and 4 show the same parts but in the intermediate and final working stages, respectively. Fig. 5 is an edge 40 view of the cold-working and shaping roller beginning operations upon the wheel blank as parted in Fig. 4. Figs. 6, 7, 8 and 9 are enlarged sectional views illustrating in detail the gradual changes which take place 45 in the final cold-rolling operations using the beveled channeled roller shown in Fig. 5.

To those skilled in the art of working copper it is well known that copper may be hardened by compression and cold working, especially if the metal is caused to flow upon itself by such compression or cold working. To effect such results in a facile and inexpensive way in making a grooved trolley wheel, I first cast or forge a solid 50 metal blank 2 of disk-shape having round

hollow hub portions 3—3 and a rounded annular swell or enlargement 4 in its body portion, see Figs. 1 and 2. This blank 2 is clamped between a pair of axially-aligned dies 5—5 having opposed beveled faces 6—6 to permit the blank to be rotated at two-hundred to three-hundred revolutions per minute opposite a pressure-applying parting roller 7. This parting roller is mounted in any suitable way and associated with means 60 adapted to force feed the roller against the periphery of the blank toward the axis of the blank and the holding dies, and in practice I use a roller 7 having beveled sides 8—8 and a rounded parting edge 9 in lieu 65 of a sharp cutting edge as shown and described in my copending application. As a result when this round-edged roller 7 is fed forward and forced into the edge of the rapidly revolving blank 2 exactly at its middle 70 the circumferential portion of the blank is parted equally. In this action the parted sides curve outwardly until the end edges engage the dies 5—5, which occurs when the roller has entered a substantial distance to 75 produce a relatively deep annular groove with a small round bottom in the blank. The rolling movement and the pressure which is applied to effect the parting causes 80 the metal in the surfaces of the groove to flow upon itself which hardens this surface and its contiguous areas, and the rounded parting edge of the roller effects a parting without splitting the disk or creating any fissure or fracture at the base of the groove. 85 Consequently, the grooved product when made in this way may be further expanded and shaped without resorting to preliminary cutting operations or removal of any of the stock at the base of the groove. 90

Thus, in practicing this process I withdraw or retire the parting roller 7 and enter a second and more obtusely beveled roller S into the parted blank while it is still clamped between the dies and under rotation, the purpose being to straighten the curved sides or flanges of the blank, to widen and reshape the groove, and to re-work metal in the surface of the groove into a harder state by crowding and flowing the 105 metal toward and into the base of the groove. In so doing I have also conceived the idea of eliminating any fault or fissure which might occur by crowding the metal on converging lines into the base of the 110

groove and producing a seam or overlap of metal which may not be manifest to the eye but if present will develop irregularities or defects eventually in the base of the groove in the trolley wheel. I accomplish the desired end by employing a reversely-beveled shaping roller S having a narrow annular space or relatively deep channel 10 at the apex of its converging sides, the summit or 10 high point at each side of the channel being rounded to produce a rounded bottom in the trolley wire groove in the wheel. The straight beveled sides of roller S flatten the curved sides or flanges of the parted blank 15 as this roller is fed under considerable pressure into the groove against such sides and as this occurs the rounded summit portions 11-11 at each side of the channel 10 in the roller crowd and roll the material in the 20 grooved surface in advance of the roller in increasing degree until this material flows toward the middle and into channel 10, as indicated in Figs. 6 to 9, inclusive where Fig. 6 shows the parted sides or flanges of the 25 wheel blank in the first stages of being flattened, and Fig. 7 shows a slightly advanced state of flattening and an initial movement of the material in the groove surface at 12 toward the channel 10. Fig. 8 shows the 30 flanges nearly flattened against the dies and the material which has been crowded and rolled downward from the sides of the groove as nearly closed together and starting to work up into the channel 10, while 35 Fig. 9 shows the flanged sides flattened and conforming to the beveled and rounded portions of roller S with a slight surplus of metal crowded into channel 10. This surplus of metal forms an annular bead or 40 ridge 14 having a crack or fissure, but this crack or fissure is located entirely within the area of the channel.

Upon withdrawing or retiring roller S from the grooved wheel, the ridge 14 is 45 easily removed by cutting, filing or grinding until the bottom of the groove is smoothly rounded. This completes the making of the wheel, excepting the boring of an opening axially for a bushing or a shaft, or some 50 other finishing step not necessarily a part of this invention, which as stated herein, consists in the main of parting the blank by applying a rolling pressure with a rounded parting roller or equivalent tool, and then 55 of expanding and reshaping the parted blank by applying a rolling pressure with a second roller and crowding the material in the sides of the grooved surface on lines moving toward the center of the bottom of the groove until a ridge or bead is formed 60 to embrace any fissure, crack or line of division produced by such crowding and flowing movement of the metal upon itself on converging lines toward the bottom and 65 center of the groove.

What I claim, is:

1. A method of making a trolley wheel, consisting in forming a deep circumferential groove in a round body of ductile metal of high electrical conductivity, in working 70 the material in the opposite faces of the groove into confluence at the bottom of the groove, and in removing the surplus confluent stock.

2. A method of making a trolley wheel, 75 consisting in parting and spreading the peripheral portion of a disk-shaped blank of ductile metal until a relatively deep circumferential groove is formed, in shaping and working the sides of the groove while 80 flowing the material in the opposite faces of the groove into raised confluence at the bottom of the groove, and in removing the raised confluent material to round the groove.

3. A method of making a trolley wheel, consisting in parting a disk-shaped blank of ductile metal by the application of a rolling pressure, in expanding and reshaping the 90 parted blank, in crowding the material in the parted faces on lines moving toward the center and bottom of the parting until a ridge of surplus material is produced, and in removing the ridge thus formed.

4. In a method of making a trolley wheel, 95 the step of crowding and flowing the material involved in the grooved faces of a trolley wheel body on confluent lines until a bead is formed embracing any fissure or line of division at the place of meeting. 100

5. A method of making a trolley wheel, consisting in forcing a round-edged roller into the peripheral edge of a disk-shaped blank of ductile metal until a relatively deep round-bottomed groove and flaring side 105 flanges are produced, then forcing a second larger roller between said flanges and crowding the material in the groove faces toward the bottom of the groove while permitting the surplus material to build up at 110 the middle of the groove, and finally in removing the surplus material and smoothly rounding the bottom of the groove.

6. A method of making a trolley wheel, 115 consisting in forcing a beveled round-edged roller into the circumference of a revolving disk-shaped blank of ductile metal until a relatively deep groove and flaring side flanges are produced; in forcing a larger beveled channeled roller between the flanges 120 of the revolving blank until a different shape is imparted thereto and the material in the opposite faces of the groove is crowded into the bottom of the groove with the surplus metal and line of meeting extending into 125 the channel in said roller; and in removing the surplus metal and rounding the bottom of the groove.

7. A method of making trolley wheels, 130 consisting; first, in forming an annular

groove in a body of ductile and tenacious metal of high electrical conductivity; secondly, in subjecting the surface of the groove to a rolling pressure moving on converging lines to crowd the material in the surface toward the center and bottom of the groove until a circumferential bead is formed embracing the meeting line of the flowing material; and thirdly, in removing the bead on rounded lines conforming to the bottom of the groove.

In testimony whereof I affix my signature in presence of two witnesses.

WILLIAM S. BIDLE.

Witnesses:

GEO. E. KRICKER,  
DOROTHY MOSER.